

## 1

2,901,312

## PROCESS UTILIZING FLUIDIZED BEDS IN THE DYING OF FABRICS, YARNS AND THE LIKE

Francis George Audas, Cheadle Hulme, England, assignor to The British Rayon Research Association, Manchester, England, a British association

No Drawing. Application May 3, 1956  
Serial No. 582,335

Claims priority, application Great Britain May 7, 1955

7 Claims. (Cl. 8—151)

This invention concerns the dyeing of filaments, fibres, threads, yarns, films and sheets of Terylene (R.T.M.), nylon, cellulose triacetate rayon or secondary acetate rayon or the like synthetic materials or of fabrics made therefrom.

Considerable difficulty has hitherto been experienced in the dyeing of Terylene and nylon and, to a lesser extent, of cellulose triacetate rayon and secondary acetate rayon or the like synthetic materials and in the fixing in reasonable times at atmospheric temperatures of a satisfactory amount of dye with the requisite uniformity and without damage to the dyed material. For example the time required for dyeing Terylene fabric or yarn with a given disperse-acetate dye, which at moderate temperatures of the order of 85° C. is excessive may be considerably reduced at temperatures of the order of 120° C. but such processing normally requires the dyeing unit to be pressurized, and this is inconvenient and adds to the expense of the process.

Considerable effort has been directed to the development of high temperature dyeing techniques which do not involve pressurization of the dyeing unit. It has been found possible for example to pass certain fabrics through a suspension of dyestuff in an aqueous bath, to dry the fabric, and then heat it to a temperature high enough to permit the padded and unfixed dye to diffuse into the fibres of the fabric material. In such methods, in order to achieve satisfactory dyeing, it is frequently necessary to use temperatures of 200° C. or more, for periods of from ten to thirty seconds. These high temperatures are disadvantageous as they tend to cause considerable shrinkage of the material. This difficulty may be overcome by prior heat setting, in conjunction with stentering at a higher temperature still but the temperatures involved might well reach a level at which the material is damaged. For example, the melting point of Terylene is only about 240° C. Stentering during the dyeing process is also likely to give rise to local temperature variations and consequent uneven dyeing.

Other attempts at overcoming these difficulties have included the addition to the dyeing bath of carriers or swelling agents but the known agents, while enabling the dyeing and fixing times and temperatures to be decreased, have suffered from the disadvantage of imparting a disagreeable odour to the material under treatment, or of impairing the light fastness of the dye, or of failing to provide the requisite uniformity of colour.

The main object of the invention is to provide an improved method of dyeing filaments, fibers, threads, yarns, films and sheets of Terylene, nylon, cellulose triacetate rayon and secondary acetate rayon and of fabrics made therefrom and we have found that this object may be achieved by the use in conjunction with certain dyeing assistants in the dyebath of the step of drying and heat treatment or of heat treatment described and claimed

## 2

in the complete specification of our co-pending application Nos. 547,681, filed November 18, 1955, and 507,705, filed March 11, 1955, and now Patent No. 2,785,478. In some cases the object may also be achieved, though to a lesser extent, if the said dyeing assistants are used with other methods of drying and heating already known in connection with the said material under treatment. These assistants are glycerine, triethanolamine, diacetin, erythritol, penta erythritol, ethylene glycol, di-ethylene glycol, di-ethylene glycol diacetate, D-glucose monohydrate, thiourea, urea, ammonium thiocyanate, hexamine, a mixture of urea and ethylene glycol, a mixture of thiourea and ethylene glycol, a mixture of penta erythritol and thiourea, a mixture of glycerine and thiourea, and a mixture of di-ethylene glycol diacetate and thiourea (hereinafter and in the claiming clauses hereof called "a defined dyeing assistant").

According to the present invention a method of dyeing filaments, fibers, threads, yarns, films and sheets of 20 Terylene, nylon, cellulose tri-acetate rayon or secondary acetate rayon or the like synthetic materials or of fabrics made therefrom comprises passing the material under treatment into a dyebath containing a defined dyeing assistant and a dye, padding the dye on to the material 25 under treatment and then passing the material under treatment through a bed of hot discrete particles, while the bed is subjected to an upward gaseous current, the size and weight of the particles, the velocity and nature of the current and the disposition of the material under 30 treatment being so chosen that the forces exerted by the current on the particles are sufficient to counter-balance the gravitational force on free particles and to expand the bed, thus allowing movement of the particles, but is insufficient to convert the bed into a uni-directional 35 stream of moving particles, and the temperature in the bed being so chosen that the dye is fixed in the material under treatment.

The nature of the said bed (hereinafter and in the claiming clauses hereof called "a fluidised bed") and the 40 manner of making the same is fully described in the specifications of the said co-pending applications.

The actual proportion of the defined dyeing assistant 45 in the bath may vary within fairly wide limits and the best proportion can easily be determined for any particular material by simple trial. It may be as low as 1% or as high as 20% but it will preferably be between 5% and 12% according to the assistant used, the percentages being by volume, or weight as the case may be, depending on whether the assistant is a liquid or a solid.

50 We have found that the present invention enables dyeing to be more readily effected than with known methods and with advantages not possessed by the known methods.

The invention will now be illustrated by the following 55 examples.

*Example 1*

Four dyebath liquors were prepared each of which contained 5% by weight of the dye Duranol Brilliant Violet 60 BR300 (C.I. 62,030) and 0.2% by weight of the wetting agent Perminol PP. One liquor contained no assistant, one contained 5% by volume of glycerine, one contained 5% by volume of diacetin, and one contained 5% by volume of triethanolamine.

65 Nylon and Terylene continuous filament fabrics were padded through the dyebath liquors, and, after mangling, were passed through a fluidised bed of sand at 195° C., the time in the bed being ten seconds. The dyed fabrics were treated with a hot soap solution to detach unfixed

dye and after rinsing and drying were analysed for dye content. The results were as follows:

| Percent by volume of dye bath assistant | Percent by weight of dye on nylon | Percent by weight of dye on Terylene |
|-----------------------------------------|-----------------------------------|--------------------------------------|
| None                                    | 1.48                              | 0.93                                 |
| 5% glycerine                            | 1.82                              | 1.34                                 |
| 5% diacetin                             | 1.99                              | 1.39                                 |
| 5% triethanolamine                      | 1.80                              | 1.15                                 |

*Example 2*

The same procedure as in Example 1 was followed except that the dyebath liquor contained 5% by weight of the dye Serisol Fast Red 3BL (C.I. 61,140) and the fabrics used were of continuous filament secondary acetate rayon, cellulose triacetate rayon, and Terylene.

The results were as follows:

| Percent by volume of dye bath assistant | Percent by weight of dye on secondary acetate rayon | Percent by weight of dye on cellulose triacetate | Percent by weight of dye on Terylene |
|-----------------------------------------|-----------------------------------------------------|--------------------------------------------------|--------------------------------------|
| None                                    | 1.19                                                | 0.55                                             | 0.31                                 |
| 5% glycerine                            | 1.50                                                | 1.33                                             | 1.27                                 |
| 5% diacetin                             | 1.46                                                | 1.16                                             | 0.95                                 |
| 5% triethanolamine                      | 1.23                                                | 1.21                                             | 1.11                                 |

*Example 3*

The same procedure as in the preceding examples was followed except that 10% by weight of Duranol Red X 3B 300 (C.I. 62,015) dye was used in the liquor, the fabrics were of continuous filament Terylene and spun Terylene respectively, and ten liquors were used, the assistants being set out in the results which were as follows:

| Percent by volume or weight (as the case may be) of dye bath assistant | Percent by weight of dye on continuous filament Terylene | Percent by weight of dye on Spun Terylene |
|------------------------------------------------------------------------|----------------------------------------------------------|-------------------------------------------|
| None                                                                   | 1.88                                                     | 2.20                                      |
| 5% glycerine                                                           | 2.49                                                     | 2.71                                      |
| 3.3% ethylene glycol                                                   | 2.15                                                     | 2.29                                      |
| 7.6% hexamine                                                          | 1.98                                                     | 2.40                                      |
| 10.9% D-glucose monohydrate                                            | 2.44                                                     | 2.42                                      |
| 4.1% ammonium thiocyanate                                              | 1.97                                                     | 2.72                                      |
| 4.1% thiourea                                                          | 2.28                                                     | 2.41                                      |
| 3.3% urea                                                              | 2.03                                                     | 2.51                                      |
| 1.65% urea K 1.65% ethylene glycol                                     | 2.05                                                     | 2.35                                      |
| 2.1% thiourea K 1.65% ethylene glycol                                  | 2.32                                                     | 2.38                                      |
| 2.5% glycerine K 2.15% thiourea                                        | 2.40                                                     | 2.83                                      |

It is to be understood that passage through the hot fluidised bed dries the fabric as well as fixes the dye when the fabric is passed straight from the dyebath to the bed as in the foregoing examples. The actual fixing time is therefore only part of the total time in the bed. For example if the total time is 10 seconds, drying may take three or four seconds, and fixing the remainder of the time. Drying need not necessarily be carried out in a fluidised bed and it is possible without serious loss of advantage to dry the material by other methods and then heat treat the material to fix the dye by passing through a fluidised bed. Likewise the increased weights of dye fixed on the material under treatment result from the use of the defined dyeing assistant and it is thus possible to obtain some of the advantages of the invention by the use of the defined dyeing assistants with other forms of drying and heat treatment. Glycerine is preferred as the defined dyeing assistant as it is cheap and easily removed from the dyed material. Other defined dyeing assistants which are also cheap and easily removed are diacetin and D-glucose monohydrate.

The process of the invention gives an increase in the

weight of dye which is fixed on a fabric for a given time and temperature of heat treatment.

What I claim is:

1. A method of dyeing filaments, fibres, threads, yarns, films, and sheets made of a synthetic fibrous material, comprising the steps of passing a synthetic fibrous material adapted to be dyed into a dye bath containing a dyeing assistant, the dye of said dye bath being adapted to be fixed at a predetermined temperature; padding said dye onto said synthetic fibrous material; and passing the thus treated synthetic fibrous material containing said dye through a bed of hot, solid, discrete particles, while subjecting the bed to an upward gaseous current, the size and weight of the particles and the velocity and nature of the current being so chosen that the force exerted by the current is sufficient to counter-balance the gravitational force on free particles and to expand the bed thus allowing movement of the particles but is insufficient to convert the bed into a unidirectional stream of moving particles, the temperature of the bed being substantially at said predetermined temperature and the rate at which said treated synthetic fibrous material is passed therethrough, being adjusted to fix said dye into said synthetic fibrous material.

2. A method of dyeing filaments, fibres, threads, yarns, films, and sheets made of a synthetic fibrous material, comprising the steps of passing a synthetic fibrous material adapted to be dyed and being selected from a group consisting of Terylene, nylon, cellulose triacetate, rayon and secondary acetate rayon into a dye bath containing a dyeing assistant, the dye of said dye bath being adapted to be fixed at a predetermined temperature; padding said dye onto said synthetic fibrous material; and passing the thus treated synthetic fibrous material containing said dye through a bed of hot, solid, discrete particles, while subjecting the bed to an upward gaseous current, the size and weight of the particles and the velocity and nature of the current being so chosen that the force exerted by the current is sufficient to counter-balance the gravitational force on free particles and to expand the bed thus allowing movement of the particles but is insufficient to convert the bed into a unidirectional stream of moving particles, the temperature of the bed being substantially at said predetermined temperature and the rate at which said treated synthetic fibrous material is passed therethrough being adjusted to fix said dye into said synthetic fibrous material.

3. A method of dyeing filaments, fibres, threads, yarns, films, and sheets made of a synthetic fibrous material, comprising the steps of passing a synthetic fibrous material adapted to be dyed and being selected from a group consisting of Terylene, nylon, cellulose triacetate, rayon and secondary acetate rayon into a dye bath containing a dyeing assistant, the dye of said dye bath being adapted to be fixed at a predetermined temperature; padding said dye onto said synthetic fibrous material; and passing the thus treated synthetic fibrous material containing said dye through a bed of hot, solid, discrete particles of siliceous sand, while subjecting the bed to an upward gaseous current, the size and weight of the particles and the velocity and nature of the current being so chosen that the force exerted by the current is sufficient to counter-balance the gravitational force on free particles and to expand the bed thus allowing movement of the particles but is insufficient to convert the bed into a unidirectional stream of moving particles, the temperature of the bed being substantially at said predetermined temperature and the rate at which said treated synthetic fibrous material is passed therethrough being adjusted to fix said dye into said synthetic fibrous material.

4. A method of dyeing filaments, fibres, threads, yarns, films, and sheets made of a synthetic fibrous material, comprising the steps of passing a synthetic fibrous material adapted to be dyed and being selected from a group consisting of Terylene, nylon, cellulose triacetate, rayon

and secondary acetate rayon into a dye bath containing a dyeing assistant, the dye of said dye bath being a disperse-acetate dye adapted to be fixed at a predetermined temperature; padding said dye onto said synthetic fibrous material; and passing the thus treated synthetic fibrous material containing said dye through a bed of hot, solid discrete particles, while subjecting the bed to an upward gaseous current, the size and weight of the particles and the velocity and nature of the current being so chosen that the force exerted by the current is sufficient to counter-balance the gravitational force on free particles and to expand the bed thus allowing movement of the particles but is insufficient to convert the bed into a unidirectional stream of moving particles, the temperature of the bed being substantially at said predetermined temperature and the rate at which said treated synthetic fibrous material is passed therethrough being adjusted to fix said dye into said synthetic fibrous material.

5. A method of dyeing filaments, fibres, threads, yarns, films, and sheets made of a synthetic fibrous material, comprising the steps of passing a synthetic fibrous material adapted to be dyed and being selected from a group consisting of Terylene, nylon, cellulose triacetate, rayon and secondary acetate rayon, into a dye bath containing glycerine as a dyeing assistant, the dye of said dye bath being adapted to be fixed at a predetermined temperature; padding said dye onto said synthetic fibrous material; and passing the thus treated synthetic fibrous material containing said dye through a bed of hot, solid, discrete particles, while subjecting the bed to an upward gaseous current, the size and weight of the particles and the velocity and nature of the current being so chosen that the force exerted by the current is sufficient to counter-balance the gravitational force on free particles and to expand the bed thus allowing movement of the particles but is insufficient to convert the bed into a unidirectional stream of moving particles, the temperature of the bed being substantially at said predetermined temperature and the rate at which said treated synthetic fibrous material is passed therethrough being adjusted to fix said dye into said synthetic fibrous material.

6. A method of dyeing filaments, fibres, threads, yarns, films, and sheets made of a synthetic fibrous material, comprising the steps of passing a synthetic fibrous material adapted to be dyed and being selected from a group consisting of Terylene, nylon, cellulose triacetate, rayon and secondary acetate rayon into a dye bath containing diacetin as a dyeing assistant, the dye of said dye bath being adapted to be fixed at a predetermined temperature; padding said dye onto said synthetic fibrous material; and passing the thus treated synthetic fibrous material containing said dye through a bed of hot, solid, discrete particles, while subjecting the bed to an upward gaseous current, the size and weight of the particles and

the velocity and nature of the current being so chosen that the force exerted by the current is sufficient to counter-balance the gravitational force on free particles and to expand the bed thus allowing movement of the particles but is insufficient to convert the bed into a unidirectional stream of moving particles, the temperature of the bed being substantially at said predetermined temperature and the rate at which said treated synthetic fibrous material is passed therethrough being adjusted to fix said dye into said synthetic fibrous material.

7. A method of dyeing filaments, fibres, threads, yarns, films, and sheets made of a synthetic fibrous material, comprising the steps of passing a synthetic fibrous material adapted to be dyed and being selected from a group consisting of Terylene, nylon, cellulose triacetate, rayon and secondary acetate rayon into a dye bath containing D-glucose monohydrate as a dyeing assistant, the dye of said dye bath being adapted to be fixed at a predetermined temperature; padding said dye onto said synthetic fibrous material; and passing the thus treated synthetic fibrous material containing said dye through a bed of hot, solid, discrete particles, while subjecting the bed to an upward gaseous current, the size and weight of the particles and the velocity and nature of the current is sufficient to counter-balance the gravitational force on free particles and to expand the bed thus allowing movement of the particles but is insufficient to convert the bed into a unidirectional stream of moving particles, the temperature of the bed being substantially at said predetermined temperature and the rate at which said treated synthetic fibrous material is passed therethrough being adjusted to fix said dye into said synthetic fibrous material.

#### References Cited in the file of this patent

#### UNITED STATES PATENTS

|           |         |               |
|-----------|---------|---------------|
| 2,080,254 | Dreyfus | May 11, 1937  |
| 2,349,282 | Kern    | May 23, 1944  |
| 2,785,478 | Audas   | Mar. 19, 1957 |

#### OTHER REFERENCES

Giradet: Industrie-Anzeiger, vol. 75, No. 12, February 10, 1953, pp. 141-143.

Saville, A.K.: "The Printing of Nylon Piece Goods," Am. Dyestuff Reporter, September 19, 1949, pp. 673-674.

45 Du Pont: "The Techn. Bull.," vol. 5, No. 2, June 1949, pp. 83-102.

Kite, R.P. and Roberts, E.J.: "Fluidization in Non-Catalytic Operations," Chem. Eng., December 1947, pp. 112-115.

50 Diserens, L.: "Les Produits Aux. dans l'Ind. Textile," Rev. Gen. Mat. Col., March 1957, pp. 89-100.

Am. Dyestuff Rep. (I), August 17, 1953, pp. 543, 544.

Am. Dyestuff Rep. (II), February 18, 1952, p. 104.